

# UNITED STATES PATENT OFFICE.

CHRISTEN JOHANNES STAUTSBOLL LUNDSGAARD, OF VEJEN, AND KAJ TOBIAS HERBST, OF BRABAND, DENMARK.

## EXPLOSIVE MATERIAL.

1,423,233.

Specification of Letters Patent. Patented July 18, 1922.

No Drawing.

Application filed September 14, 1921. Serial No. 500,663.

*To all whom it may concern:*

Be it known that we, CHRISTEN JOHANNES STAUTSBOLL LUNDSGAARD and KAJ TOBIAS HERBST, subjects of the King of Denmark, 5 residing at Vejen, Denmark, and Braband, Denmark, respectively, have invented new and useful Improvements in Explosive Materials; and we do hereby declare the following to be a full, clear, and exact description 10 of the same.

The object of the invention is to provide an explosive which has a high explosive power and a high degree of stability and which advantageously may be used for any 15 military or civil purpose where explosives are employed.

Another object of the invention is to provide an explosive of the kind described which which shall be substantially insensible 20 against moistness.

A further object of the invention is to provide a detonator containing our new explosive.

With these and other objects in view the 25 explosive consists of or comprises a perchlorate of a methyl-substituted ammonium compound.

It is a well known fact that efficient and stable explosives can be produced by the action 30 of perchloric acid or perchloric compounds upon cyclic ammonium compounds. It has also been tried to produce perchlorates of alifatic amino compounds, viz, ethylenediamine and dicyan-diamine, for explosive 35 purposes, but so far as we are aware these substances have not been used in large scale due to their hygroscopic character and high costs of production. It has now been found in practice that efficient and stable explosives

40 can be obtained by the action of perchloric acid or perchloric compounds upon methylamine, dimethyl-amine, trimethyl-amine, tetramethyl-ammonium or compounds containing one or more of said substances, 45 whereby the corresponding perchlorates are formed. Said perchlorates are rather insensible against moistness except the perchlorate of dimethyl-amine. Thus the perchlorate of methyl-amine certainly is freely

50 soluble in water, but it is only slightly hygroscopic, while the perchlorate of tetramethyl-ammonium dissolves with difficulty in water. Moreover these substances are

very stable. Thus they may be subjected to a temperature of 150° C. for a long period 55 and they may be stored for several years without decomposition. An explosive of the kind described which has an especially high explosive power is the perchlorate of methyl-amine. Said substance may be produced, say by neutralizing dilute perchloric acid by a solution of methylamin and subsequent vaporization and crystallization. It is found in practice that 0.25 g. of the resulting perchlorate compressed in a 65 copper cap by a pressure of 1500 kg. pr. cm<sup>2</sup> and ignited by a charge of 0.4 g. mercuric fulminate forms a hole of a diameter of about 8-9 mm. in a lead plate of 7 mm. thickness, when the cap is disposed vertically 70 upon the surface of the lead plate. This experiment shows that the substance in question has an exceptional brisant action and efficiency which partially is due to its rather ideal composition with respect to 75 the proportions of the carbon, hydrogen and oxygen content. Furthermore this perchlorate can be produced at low costs, since the methyl-amine may be easily obtained by hydrogenation of hydrocyanic acid or by 80 distillation of sugar residues. This explosive may therefore successfully be employed for military and civil purposes (as charge for mines, shells etc. or as explosive for mining and the like purposes) either in pure 85 state or in mixture with other substances. Preferably the new explosive may be used as an admixture to well known explosives, whereby the efficiency of the latter is increased. 90

Moreover the new explosive may advantageously be used as an intermediate charge in detonators, exploders or the like. Furthermore the pure explosive or mixtures of the same may be mixed with carbonates or 95 hydroxydes of sodium, calcium, magnesium or the like in order to neutralize the acid combustion products which are formed by the explosion.

Having thus fully described our invention 100 we claim as new and desire to secure by Letters Patent:

1. An explosive comprising a perchlorate of methyl-substituted ammonium compound.
2. An explosive comprising a compound 105 produced by the action of a perchloric com-

pound upon a methyl-substituted ammonium compound comprising at least one methyl group.

3. An explosive containing mono-methyl-  
5 ammonium-perchlorate.

4. An explosive comprising a perchlorate  
of a methyl-substituted ammonium com-  
pound and a substance for neutralizing  
acidulous combustion products.

0 5. A detonator containing a perchlorate

of a methyl-substituted ammonium com-  
pound.

In testimony whereof we have affixed  
our signatures in presence of two witnesses.

CHRISTEN JOHANNES STAUTSBOLL LUNDSGAARD.  
KAJ TOBIAS HERBST.

Witnesses:

FANNY GESERSEN,  
C. V. HOGE SEE.